

## UNITED STATES PATENT OFFICE.

ALBERT C. FISCHER, OF CHICAGO, ILLINOIS.

## EXPANSION JOINT.

No Drawing.

Application filed May 3, 1926. Serial No. 106,561.

My invention relates in general to expansion joints, and has particular reference to expansion joint materials for use in concrete or the like constructions, particularly concrete road construction, bridges, breakwaters, and other like constructions in which expansion and contraction of the concrete is to be provided for by expansion contraction joint material, arranged in the form of strips 10 at spaced intervals in the concrete structure.

These expansion contraction joints are usually provided in either of two ways. One way being to leave a space between sections of the concrete with the space filled with 15 the joint material by pouring. Another way being to furnish premoulded or preformed strips of joint material with the same installed between the concrete sections. Usually the strip is supported on edge and the 20 concrete sections poured against opposite sides of the same, so that it practically forms an inseparable part of the sections, i. e. to say a provision is made to insure the bond between the sides of the joint and the concrete 25 sections.

Owing to the service that the joint is intended to perform and the difficulties to be expected in the performance of the joint unusual care and scientific preparation of the 30 joint is of the utmost importance. Since practically all concrete constructions are built according to specifications, which also embrace the joint material, it is necessary to construct the joint to meet these specifications, otherwise the material is not acceptable. As an example, most joint material is provided in the form of strips, the dimensions of which range from  $\frac{1}{4}$  inch to 2 inches in thickness and usually in lengths of 5 to 15 35 feet, the width of the strip being the depth of the wall surface or slabs between which the strips are placed. These same dimensions apply for the most part to poured joints as well as to moulded joints, in other words, in the 40 case of a poured joint a space is left so that the joint when poured will be of a dimension required under the specifications.

Before the joint is installed in the concrete it must pass certain severe tests. As an example, the requirements for one of these tests calls for a material which will withstand the effect of what is known as a test for brittleness. In this test a piece of joint about 6 inches square must not shatter or crack at 45  $40^{\circ}$  F., so that in cold weather the joint will not become brittle or fail to function prop-

erly. As another extreme the joint must also perform properly at higher temperatures, ranging from  $70^{\circ}$  to  $115^{\circ}$  F. From the above it will be seen that the joint is called upon to 60 function properly at one extreme temperature as well as another extreme. These severe tests make it necessary to go to considerable expense in providing a material which will be acceptable, and these requirements, as 65 above stated, are often difficult to overcome.

The primary object of my invention is to provide a joint or joint material which will meet the requirements and properly function at all times. To accomplish this purpose I have selected various materials which enter in the composition of the joint, the material being used selectively or collectively for certain specific reasons, and prepared in a particular manner as will hereinafter follow.

The object of an expansion joint is to compensate for the expansion and contraction of the concrete sections. At warm temperatures the concrete expands, which means that this 80 expansion must be compensated for by the joint. In other words, the joint will be subjected to severe pressure from the sides, and unless the joint is properly prepared, the tendency is for the material to ooze out of the 85 joint and spread itself on the surface of the road, where it will be picked up by passing traffic and spread over the road. According to my invention I can prevent this oozing of the joint, and one of the objects of the same 90 is to accomplish this end.

In cold weather when the concrete sections contract the tendency is, of course, to leave a larger space in the joint. Consequently, unless the joint material has the inherent 95 quality of expanding from within it will not fill up this enlarged space in the joint. Another object of my invention is to provide a joint material which will expand from within so as to keep the space in the joint filled at 100 all times.

The matter of elongation of the joint strip is also taken into account. When the concrete sections expand and the pressure is imparted to the sides of the joint, the joint has 105 a tendency, as above stated, to ooze, and it also has a tendency to become elongated. As another object of my invention I propose to overcome this defective elongating of the joint, due to pressure on the sides.

Still another object of my invention is to provide a joint which in the case of a pre-

formed strip may be handled properly on the job, may be stored without wilting, so to speak, and which may be laid so as to leave a straight edge, that may be made by an economical method and offered for sale at a moderate price.

With these and other objects in view, as will appear as the description now proceeds, I will first describe the materials entering into 10 the manufacture of the joint and the function of the same when used selectively or collectively.

Owing to its inherent compressibility, resiliency and ductile qualities I prefer to use 15 bituminous matter as a base for the composition of which the joint is produced, and more particularly I would prefer to use blown asphalt, as bituminous matter in this form serves the purpose to best advantage, primarily owing to the fact that it retains its 20 resiliency, compressibility and ductile qualities after it has cooled off and has been moulded into a strip.

While, as stated bituminous matter in the 25 form of blown asphalt is preferred, I do not wish to be limited to the use of this particular material as it is possible some other waterproofing material having the same characteristics may prove just as acceptable. In 30 any event, considering the base of the composition as comprising a waterproofing material having inherent compressibility and resiliency, and using blown asphalt as an example, I will proceed in producing material as 35 follows:

By simply using a strip of bituminous matter, even blown asphalt, certain difficulties 40 will arise which prohibit the joint being made with this material alone. In the first place, if it were made hard enough to handle properly it would be too brittle to compensate for expansion, and could not be properly handled in cold weather, as it would easily crack and even break. If it were made soft 45 enough so as to compensate for expansion of the concrete, it would not only ooze out of the joint but in warm weather it would turn into practically a semi-fluid, in fact it would be out of the question to use this material without 50 the aid of other materials to overcome these defects.

To overcome these conditions I propose to use certain materials in combination with a binder or base, as I have referred to it, so as to 55 make it practically what in effect is a composition of matter comprising a binder and a frame structure within the binder, with this frame structure reinforced or strengthened, and in addition a filler. This composition 60 can be likened in many respects to the same theory as that concerned with the reinforcement of concrete. In other words, I incorporate a binder with the material which will build up a frame structure, with the frame 65 structure reinforced by a different class of

material and the whole increased in bulk by still another class of material. These three different groups of materials may be used with the binder selectively or collectively, in order to produce a joint material that will 70 meet certain requirements.

As a more specific embodiment of the composition I will classify the materials in groups, for instance, group A is a binder, such as blown asphalt or any other suitable waterproofed material. This binder will form the bulk or base of the joint material and serve 75 to bind the other materials so that the composition may be formed into strips, or in some instances poured into a mould. 80 The purpose of the binder being to hold together the other materials used, to thoroughly waterproof the other materials, and to form itself under the motion of the concrete sections, and to adjust itself under pressure of 85 traffic so that it will work back into the joint and not permit itself to be carried away by traffic.

Group B, which is a frame building structure, preferably comprises such fibrous matter as bulk vegetable binder, flat grasses, blades, fronds, roofing tabs, cypress bark, eucalyptus bark, bast, also similar binding strips, such as, flat strips of paper, flat excelsior, cloth and other flat materials having 90 length. In other words, any material of the class described which will build up a framework structure in the binder. The purpose of this framework is to enable the strip to be handled without bending, wilting or 95 slumping, and to prevent the binder from oozing in warm weather and becoming too brittle and shattering or cracking in cold weather.

Group C, which is a reinforcing structure, acts somewhat the same as the framework structure, except that the materials used in this group go further, due to their inherent strengthening qualities which reinforce the composition. For this group I prefer to 100 select such fibres as cocoanut, sisal, hemp, mosses, jute or any other similar long fibre of strong quality which provides a relatively long, strong and tough fibrous material, having 105 a surface slightly roughened or otherwise formed so as to allow the binder to again a thorough hold upon the fibre. As an example, while the material classified in group B, in some respects will enable the binding material to form a bond therewith, 110 it may not have enough strength or long enough surface area to form the right kind of a bond under certain conditions. At temperatures around 70° F., if the binder does not have a thorough hold upon the fibre 115 the tendency is for the fibres to slip, so to speak, in the binder. By using such fibres as classified in group C I am enabled to overcome this possibility.

As a second group coming under the head- 120

ing of reinforcing or strengthening mediums, which may be used selectively or collectively with group C, I suggest group D, which consists of such fibrous matter as hog hair, 5 cattle hair, horse hair, and other like strong fibre having a glossy and smooth surface, which will resist pull increasingly at reduced temperature. Hair at warmer temperatures will slip through the binder, but 10 when the binder contracts and becomes set it grips the hair and the hair does not slip thru the binder. This is a particularly favorable material for use at temperatures ranging from 32° to 60° F. It also imparts resiliency and takes up shock in the material. 15 It is a deciding factor at low temperatures, while the material in group C is a deciding factor at high temperatures. In other words, for joint materials that are to be used al- 20 most exclusively at higher temperatures I would suggest the use of materials classified in group C, and for joint material that was to be subjected to lower temperatures I would suggest the use of the material referred to in group D. As stated, the materials in groups C and D may be used selectively or collectively.

As a filler to add bulk to the mass and reduce the weight of the binder I will classify 30 the following materials as group E, the same consisting of such materials as cotton waste, shoddy, roofing scrap and other finely divided ultimate fibres, such as, wood pulp, these materials to be utilized for the purpose 35 of making up bulk. These materials will provide a fibrous filler of very short lengths distributed throughout the binding material, which will make the binder more sluggish and resist its tendency to flow under 40 pressure. As a matter of fact the materials classified in group E are in one sense a flow controlling substance, and they would hardly ever be used singly, that is to say, with simply a binder without the materials classified 45 in groups C and D. They may be used in combination with either of the materials used in group C or D, or with both groups of materials.

As a further group of materials to be used, 50 viz, group F, I would classify limestone dust, talc, mica, asbestos fibre or clay, mostly all in the form of dust, which are placed upon the surface of the material to prevent adhesion or to function in various ways as 55 a coating for the outside of the material.

As an alternative coating medium in the composition I will refer to group G, containing a latex wash, gelatine, glycerine wash, polymerized oil, coating, gluten-gly- 60 cerine, a rubber solution, etc. The purpose of these materials being to take up surface shocks.

To make up the composition I will ordinarily proceed as follows: The binding material, such for instance, as asphalt, would

be melted down to a proper consistency so that it could be worked in a mechanical mixer. The materials classified in group E would then be incorporated, then the materials classified in groups C and D. As a 70 matter of fact it does not make much difference in which order the materials are incorporated. After the mixing thoroughly and without undue loss of time, I would reduce the mass to sheets by subjecting the 75 same to the action of sheet forming rolls, and thereafter cutting the sheets into strips. As an alternative method I could extrude the material into strips by a suitable extruding 80 machine.

The proportions of the material used are more or less important, for instance, the specifications for expansion joint material call for a preponderance of binding material, such as asphalt. To meet these requirements a suitable formula for this composition would be seventy-five (75) per cent binding material, fifteen (15) per cent of a material classified in group B, three (3) per cent of a material classified in group C, two (2) per cent of a material classified in group G and five (5) per cent of a material classified in group E. The material classified in group F may be used as a coating, and is simply dusted on the sides of the joint. In using any of the materials classified in group G as a coating the same are applied as a film or layer, as desired. 95

As a specific example of a given mixture I refer to 50 to 60 lbs. of flat excelsior, 20 to 100 10 lbs. hemp or equivalent, 50 to 40 lbs. roofing scrap, 300 to 280 lbs. bituminous material.

These proportions are simply illustrative of the possibilities. I have, of course, simply given the same as examples, and I do not care 105 to be limited to the proportions named. In any event, however, I would always use a larger percentage of binding material than any of the filling materials.

The two groups of reinforcing material 110 may be more specifically referred to, for instance, group C as a high temperature resisting material and group D as a low temperature resisting material.

I claim:

1. A preformed expansion joint comprising a ductile, compressible binder, in which the binder predominates in the excess of sixty per cent, and relatively rigid flat linear fibres, relatively long, tenuous, vegetable fibres, relatively long animal hair and a flow controlling substance, all incorporated in the bituminous material. 120

2. A preformed expansion joint comprising a ductile, compressible binder, in which the binder predominates in excess of sixty per cent, and flat linear elements composed of fibers and relatively long, tenuous, vegetable fibres incorporated therein, the former providing a rigid structural frame and 125 130

the latter providing binding strength pronouncedly effective at high temperatures.

3. A preformed expansion joint comprising a ductile, compressible binder, in which the binder predominates in excess of sixty per cent, flat linear elements forming a frame-building structure and relatively long animal hair, the animal hair providing an effective binding medium when the binder is at low temperature.

4. A preformed expansion joint mixed in the following proportions: 280 to 300 lbs. of bituminous material, 40 to 50 lbs. of roofing scrap, 10 to 20 lbs. of long tenuous vegetable fibre, such as cocoanut fibre, 50 to 60 lbs. of flat excelsior.

5. A preformed expansion joint comprising bituminous material in excess of sixty

per cent, flat linear material providing a rigid structural binder and two additional reinforcing means, each formed of relatively long, tenuous elements, one being particularly effective as a binding medium at high temperatures and the other being particularly effective as a binding medium at low temperatures.

6. A preformed expansion joint for concrete construction, comprising a ductile, compressible binder in excess of sixty per cent, relatively rigid, flat, reinforcing elements composed of fibers and long vegetable fibres and long animal hair.

Signed at Chicago, Illinois, this 1st day of May, 1926.

ALBERT C. FISCHER.